

## 1

3,576,712

**SIZING PAPER WITH EITHER SULFONE, SULF-  
OXIDE OR SULFIDE AND A POLYALKYLENE-  
IMINE**William Robert Hine, Jr., Kirkwood, and Myron J. Holm,  
St. Louis, Mo., assignors to Monsanto Company, St.  
Louis, Mo.No Drawing. Continuation-in-part of abandoned application  
Ser. No. 520,639, Jan. 14, 1966. This application  
Apr. 16, 1969, Ser. No. 816,772

Int. Cl. D21h 3/40; D21d 3/00

U.S. Cl. 162—168

8 Claims

**ABSTRACT OF THE DISCLOSURE**

A combination of a 2-chloroalkyl sulfone, a 2-chloroalkyl sulfoxide or a 2-chloroalkylsulfide, and a polyalkyleneimine which is useful as a sizing agent in the preparation of sized cellulosic paper substrates.

This application is a continuation-in-part of application Ser. No. 520,639, filed Jan. 14, 1966, and now abandoned.

This invention relates to the sizing of cellulose paper substrates. More particularly this invention provides new combinations of materials which are very effective as sizing agents under acid, neutral and alkaline pH conditions to give permanent sizing under conditions which are compatible with present papermaking procedures.

An object of this invention is to provide a combination of chemical ingredients which will size paper under a variety of pH conditions to give permanent sizing while being compatible with present papermaking procedures.

Briefly, it has been found that fibrous materials, particularly fibers of cellulose and the like, may be sized by applying to the fibrous material a combination of (a) a compound of the formula



where R is any organic hydrocarbon hydrophobic group, and R' is hydrogen, methyl, or chloromethyl and n is an integer of from 0 to 2 (b) a polyalkyleneimine having from 2 to 3 carbon atoms in each alkylene group, and thereafter drying the thus treated fibrous material. This combination of the 2-chloroalkyl sulfone, sulfoxide, or sulfide, and the polyalkyleneimine may be applied by any convenient method known to those skilled in the sizing art. They may be combined in one solution or dispersion and added to an aqueous fibrous slurry or pulp slurry, or they may be sprayed on to a fibrous mat or paper web. They may also be applied by tub sizing methods by passing cellulose containing webs or textiles through solutions of the combined ingredients or through separate solutions of the two ingredients to effect contact of the cellulosic fiber material with both of the 2-chloroalkyl sulfur compound and the polyalkyleneimine. Generally, the combination of the 2-chloroalkyl sulfone, sulfoxide or sulfide, and the polyethyleneimine is applied in combined amounts of the two ingredients sufficient to impart from about 0.01 to about 5% or more of the weight of the dry cellulose fibers.

A preferred example of the application is to add to the aqueous pulp slurry used to make cellulose containing paper, either separately or in combination a higher alkyl 2-chloroethyl or 2,3-dichloropropyl sulfone and a polyethyleneimine, the combined amounts of the two ingredients being between about 0.1 percent to about 5.0 percent of the weight of the dry pulp fiber in the pulp slurry being treated, although total percentage amounts may range from about 0.1 percent to any higher amount dic-

## 2

tated only by cost. The two ingredients are preferably combined in weight ratios of about 1:1 to 1:3 of the 2-chloroalkyl hydrophobic sulfone; polyethyleneimine although suitable weight ratio proportions may range from about 1:10 to about 10:1 and still get a sizing effect. A minimum of about 0.2% of each component should be used for effective sizing. The 2-bromoalkyl sulfides, sulfoxides and sulfones could also be used, if desired.

In another preferred aspect of this invention the sizing agents may be applied as a surface size to previously formed, untreated fibrous mats or cellulose containing webs. The combined amounts of the two aforementioned ingredients in this aspect of the invention are generally between 0.02% to about 5.0% of the weight of the dry

cellulose fibers. However, higher concentrations of the ingredients may be applied if desired, but for most practical purposes, higher concentrations are generally not needed. In this aspect of the invention the two ingredients are preferably combined in weight ratios of about 1:1 to 1:3 of the 2-chloroalkyl hydrophobic sulfone; polyethyleneimine although suitable weight ratio proportions may range from about 1:10 to about 10:1 and still attain a sizing effect. The 2-bromoalkyl sulfides, sulfoxides and sulfones could also be used in this aspect of the invention.

The effect of this particular combination of a 2-chloroalkyl sulfone, sulfoxide, and sulfide and a polyalkyleneimine is quite unexpected because combination of related materials such as 2-hydroxyethyl octadecyl sulfone with polyethyleneimine and applied in a manner similar to the application of 2-chloroethyl octadecyl sulfone and polyethyleneimine gave essentially no sizing. However, we have found that 2,3-dichloropropyl hydrophobic hydrocarbon sulfides and sulfoxides can be used to effect sizing in accordance with this invention or to replace a part or all of the corresponding sulfone in the sizing combination but the sulfone is preferred because it is more effective in this combination. The 2,3-dichloropropyl hydrophobic sulfide is much more effective in this sizing combination than is the 2-chloroethyl hydrophobic sulfide. When the 2-chloroalkyl sulfides and sulfoxides are used, however, it is usually necessary to cure the treated cellulosic material, e.g., at 105° C. for 1 hour, to effect the sizing. The corresponding sulfones in this combination effect sizing without a prolonged curing step and hence the sulfones are preferred.

The 2-chloroalkyl hydrophobic sulfides, sulfoxides, and sulfones which we have found to be useful for sizing fibrous materials, particularly cellulosic fibrous materials include those in which the hydrophobic group is a higher alkyl having at least about 10 carbon atoms, e.g., decyl, undecyl, dodecyl, tridecyl, tetradecyl, pentadecyl, hexadecyl, heptadecyl, octadecyl, tetracosyl, and pentacosyl and higher alkyl up to about 40 carbon atoms if desired, although those having up to about 25 carbon atoms are preferred, the corresponding alkenyl groups having from 10 to about 40 carbon atoms, a few examples of which are decenyl, tridecenyl, heptadecenyl, octadecenyl, eicosenyl, tricosenyl, etc., the alkylphenyl and alkyl-substituted cycloalkyl having at least about 8 carbon atoms in the alkyl groups attached to the phenyl or cycloalkyl group, e.g., octylphenyl, dinonylphenyl, dodecylphenyl, tridecylphenyl, pentadecylphenyl, octadecylphenyl, heneicosylphenyl, nonylcyclopropyl, dodecylcyclobutyl, tridecylcyclopentyl, tetradecylcyclohexyl, pentadecylcycloheptyl, octadecylcyclohexyl, etc., and any of such alkyl, alkenyl, alkylphenyl and alkylcycloalkyl, 2-chloroalkyl sulfide, sulfoxide, or sulfone compounds containing non-interfering inert substituents. Inert substituents which may be present include groups such as carboalkoxy, alkyloxy, aryloxy, arylalkyloxy, keto(carbonyl), tertiary amide, halogen attached to aromatic carbons, or aliphatic hetero-

cyclic groups, i.e., heterocyclic radicals containing no benzene-type unsaturation. The heterocyclic radical may be saturated or unsaturated. Types of radicals which should not be present to any substantial extent in the hydrophobic group are exemplified by hydroxyl groups, primary and secondary amino groups, labile halogens, amide groups having amido hydrogen, and carboxyl or other acidic groups. Those skilled in the art will be aware of the types of hydrophobic groups which may be used in these 2-chloroalkyl sulfide, sulfoxides, and sulfone compounds if undesired side reactions are to be avoided.

These sulfide, sulfoxide and sulfone compounds can be used as single pure compounds for the purpose of this invention. However, in commercial practice, 2-chloroalkyl sulfide, sulfoxide and sulfone compounds containing, e.g., mixed hydrophobic alkyl, mixed alkenyl and alkyl, alkylphenyl, or alkyl, and alkyl-substituted cycloalkyl groups may conveniently be used. Mixtures of sulfides, sulfoxides and sulfones are also useful.

For some applications of these combinations of materials to some cellulosic fibrous materials, increased sizing effectiveness is noted when these 2-chloroalkyl sulfide, sulfoxide and sulfones are applied to the fibrous substrate admixed with or simultaneously with a basic material such as an alkali metal hydroxide in an amount sufficient to effect the sizing on the basic side of the pH range, that is, about pH 7 either prior to or simultaneously with the addition of the polyethyleneimine. When this procedure is contemplated the base will usually be sodium hydroxide because it is most readily available and the most economical one to use. However, it is understood that other basic materials such as potassium hydroxide, lime, hydrated lime, calcium hydroxide, and other alkali metal and alkaline earth metal bases and basic salts could be used if desired.

The combination of the sulfide, sulfoxide and sulfone materials and the polyethyleneimine may be applied to fibrous substrates to impart sizing thereto in any conventional manner. The fibrous material in the form of cellulosic pulp, finished paper sheets or paper board, or paper product, textile fiber, thread, yarn, or fabric may be simply dipped into a water-immiscible organic solvent solution of the 2-chloroalkyl sulfide, sulfoxide, or sulfone, and then

The combination of the sizing ingredients of this invention may also be used in conjunction with starches such as "Stayco A," an oxidized corn starch by A. E. Staley Mfg. Co., when the sizing ingredients are applied to the cellulosic fibers by surface sizing techniques.

5 The polyalkyleneimines used in this invention are the polymerization products of ethyleneimine or derivatives thereof. Those used in this invention are those having from 2 to 3 carbon atoms in each alkylene group which are water soluble. Such products are described, for example, in U.S. Pat. 2,192,306. The poly(N-methylalkyleneimines) which may also be used are the polymerization products of N-methyl-ethyleneimine, N-methyl-propyleneimine, or mixtures thereof.

10 15 The following examples will further illustrate the nature of the invention but the invention is not intended to be restricted thereto.

#### EXAMPLE 1

This example illustrates the substantially enhanced 20 sizing effectiveness obtained by using the combination of polyethyleneimine and a 2-chloroethyl sulfone of the type provided for by this invention, as compared to a 2-hydroxy ethyl sulfone.

For this example, polyethyleneimine was added to a 25 2% paper pulp slurry in water in amount to equal 1% based on the dry weight of the pulp in the slurry, stirred for 15 minutes, and then 1% based on the weight of the pulp, of either 2-hydroxyethyl octadecyl sulfone as a solution in xylene or 2-chloroethyl octadecyl sulfone as a 30 solution in p-cymene was added which were emulsified in water using hexadecyltrimethyl ammonium bromide (Arquad) as an emulsifying agent. After stirring to obtain uniform dispersion, the treated pulp was formed into paper sheets on a Noble and Wood paper making machine. The paper sheets obtained were dried and some sheets were cured for 1 hour at 105° C. and tested for 35 sizing effectiveness using the ink penetration test method using seconds of time before ink is observed on the upper observed surface as the measure of sizing. Some finished 40 paper sheets were left unwashed while others were soaked in chloroform, dried and then tested for sizing in the same manner. The results of the tests are summarized in the following table.

| Agent used                                                         | Amount, percent | Cured 1 hour/105° C. |        | Sizing (sec.) |        |
|--------------------------------------------------------------------|-----------------|----------------------|--------|---------------|--------|
|                                                                    |                 | Unwashed             | Washed | Unwashed      | Washed |
| A... {Polyethyleneimine.<br>2-hydroxyethyl octadecyl sulfone.----- | 1               | No.....              | 0      | 0             | 0      |
| B... {Polyethyleneimine.<br>2-chloroethyl octadecyl sulfone.-----  | 1               | Yes.....             | 9      | 9             | 0      |
| C... Polyethyleneimine.-----                                       | 1               | No.....              | 7,000+ | 9,000+        | 0      |
|                                                                    | 1               | Yes.....             | 7,000+ | 7,000+        | 0      |
|                                                                    | 1 {No.....      |                      | 0      |               | 0      |
|                                                                    | 1 {Yes.....     |                      | 1      |               | 1      |

#### EXAMPLE 2

55 60 65 To an aqueous slurry containing 2 percent by weight of a bleached Gatineau sulfite pulp refined to a Canadian Standard Freeness of about 500±20 ml. and having a pH of 9.0 there was added an emulsion prepared by dissolving 0.75 g. of 2,3-dichloropropyl n-octadecyl sulfide or sulfone in 5 ml. of xylene and mixing with the resulting solution 20 ml. of a solution of 0.1 percent hexadecyltrimethyl ammonium bromide in water. The treated aqueous pulp slurry was mixed for 15 minutes to insure uniform distribution, and then used to make paper sheets on a Noble and Wood paper making machine. Some sheets were merely dried and then tested for sizing. Other sheets were cured for 60 minutes at 105° C. and then tested.

70 Other batches of the same bleached Gatineau sulfite pulp slurry at pH 9 were treated first with an aqueous slurry of a polyethyleneimine, mixed as before, and with one of the 2,3-dichloropropyl n-octadecyl sulfide or sulfone emulsions, as above. The resulting treated pulps were formed into sheets as above, and either dried or cured at 105° C. for 60 minutes as above, and then tested for

into a solution of the polyethyleneimine and then dried in any convenient manner. The term "drying" and its various adjective, verb, and particle forms, are used herein to include curing of the treated fibrous substrate to give a finished sized fibrous product. The amount of the 2-chloroalkyl sulfide, sulfoxide, or sulfone and the polyethyleneimine retained by the fibrous substrate can be controlled by the concentration of the treating solution and the degree of squeezing or pressing of the dipped fibrous material before drying.

This invention also contemplates the use of this combination of sizing ingredients in conjunction with agents designed to increase retention of the sizing agents on the fibrous substrate such as cellulosic fibers. Useful auxiliary agents of this type include cationic starch, a good example of which is a modified corn starch having a nitrogen content of about 0.25 percent, sold under the trade name "Cato 8" by National Starch Products Company. When from 0.1% to about 0.5% by weight, based on the weight of the fibrous substrate, e.g., cellulose pulp, of a cationic starch, such as "Cato 8" is added to the stock slurry before, after, or simultaneously with the sizing agent, a decided improvement in retention of the sizing agent is obtained.

sizing effectiveness by the ink test method. Some samples were washed with acetone, dried, and then tested to determine permanency of sizing. The results of these tests on the various papers is summarized in the following table.

| Agent used                                                                    | Amount, percent | Cured 1 hour/105° C.  | Sizing (sec.)   |                 |
|-------------------------------------------------------------------------------|-----------------|-----------------------|-----------------|-----------------|
|                                                                               |                 |                       | Unwashed        | Washed          |
| D... 2,3-dichloropropyl n-octadecyl sulfide...                                | 1               | {No-----<br>{Yes----- | 0<br>600        | 750             |
| E... 2,3-dichloropropyl n-octadecyl sulfone...                                | 1               | {No-----<br>{Yes----- | 0<br>0          | -----           |
| F... {2,3-dichloropropyl n-octadecyl sulfide...<br>{Plus polyethyleneimine... | 0.5             | No-----<br>Yes-----   | 0<br>16,000+    | 6,000+          |
| G... {2,3-dichloropropyl n-octadecyl sulfone...<br>{Plus polyethyleneimine... | 0.5             | No-----<br>Yes-----   | 2,825<br>6,000+ | 2,400<br>6,000+ |

<sup>1</sup> 6,000+ means that the test was concluded at 6,000 seconds and is indicative of hard sizing.

### EXAMPLE 3

This example illustrates the enhanced sizing effectiveness obtained by using the combination of polyethylene-imine and a 2-chloroethyl sulfone as a surface size.

#### Unsized paper preparation

Equal parts by weight of bleached softwood kraft pulp and bleached hardwood kraft pulp were slurried and refined to a Canadian Standard Freeness of 375. No pulp additives were used. The pH of the slurry was adjusted to 7.0 and the pulp was sheeted and dried on a Fourdrinier paper machine. The resulting unsized sheets had a basic weight 44 lbs./3300 sq. ft. and a Gurley porosity of 10 seconds.

#### 2-chloroethyl sulfone emulsion preparation

"Cato 8" cationic starch (National Starch Co.) in an amount of 4.5 grams and 0.34 gram of sodium lignosulfonate are mixed with 150 ml. of water and cooked at 90 to 95° C. for about 15 minutes. The mixture is then placed in a Waring Blender and 9.0 grams of 2-chloroethyl n-octadecyl sulfone is added with slow agitation and the mixture is held at a temperature of about 85° C. The resulting mixture is agitated with full speed on the blender for about 5 minutes. The resulting emulsion is poured over 100 grams of ice and then further adjusted to 300 grams with the addition of more ice. The resulting emulsion contains 3.0 of the 2-chloroethyl n-octadecyl sulfone.

#### Size press solution preparation

A 10% slurry of "Stayco A" (an oxidized corn starch of A. E. Staley Mfg. Co.) is cooked for about 15 minutes at 90 to 95° C. diluted to form a 6% solution and cooled to room temperature.

A series of size press solutions were prepared using in each solution 100 grams of the "Stayco A" solution and sufficient amounts of the sulfone stock solution and 1% polyethyleneimine solution to provide the desired final concentration of sizing compositions on each sheet based on the dry weight of the fibers as shown in the table below.

The sheets were dipped into the size press solutions and run between the rolls of a wringer and dried on a drier at 204° F. for about 30 seconds.

Results of the sizing tests on the various papers is summarized below.

| Sizing Composition on Sheet<br>Based on Weight of Dry Fibers |                                   | Sizing (sec.)                          |                                  |                                  |
|--------------------------------------------------------------|-----------------------------------|----------------------------------------|----------------------------------|----------------------------------|
| Percent<br>2-chloroethyl<br>n-octadecyl<br>sulfone           | Percent<br>polyethylene-<br>imine | Cured<br>overnight<br>at room<br>temp. | Cured<br>5 minutes<br>at 120° C. | Cured<br>5 minutes<br>at 120° C. |
| H.... .02                                                    | 0.02                              | 89                                     | 253                              |                                  |
| I.... .027                                                   | 0.027                             | 1515                                   | 1475                             |                                  |
| J.... .034                                                   | 0.034                             | 1875                                   | 1625                             |                                  |
| K.... .034                                                   | 0.100                             | 2100                                   | 1925                             |                                  |
| L.... .034                                                   | 0.013                             | 65                                     | 21                               |                                  |

What is claimed is:

1. A fibrous product comprising cellulose fibers having distributed on their surface (a) a compound of the formula



wherein R is an organic hydrophobic hydrocarbon group, R' is selected from the group consisting of hydrogen, methyl, and chloromethyl, and n is an integer of from 0 to 2, and (b) a polyalkyleneimine having from 2 to 3 carbon atoms in the alkylene groups, the combined amounts of (a) and (b) being about 0.01% to about 5% of the weight of the dry cellulose fibers, and the weight proportions of (a) to (b) being from about 1:10 to 10:1.

2. A fibrous product as described in claim 1 wherein the cellulose fibers are the type used to make paper webs, the compound (a) is one in which R is an alkyl group having at least 10 carbon atoms, R' is hydrogen, and n is 2, and (b) is polyethyleneimine.

3. A fibrous product as described in claim 2 wherein the compound (a) is 2-chloroethyl octadecyl sulfone.

4. A fibrous product as described in claim 1 wherein the cellulose fibers are the type used to make paper webs, the compound (a) is one in which R is an alkyl group having at least 10 carbon atoms, R' is chloromethyl, and n is 2, and the polyalkyleneimine (b) is polyethyleneimine.

5. A fibrous product as described in claim 4 wherein the compound (a) is 2,3-dichloropropyl octadecyl sulfone, and the compound (b) is polyethyleneimine.

6. A method of preparing a treated fibrous product of cellulosic fibers which comprises applying to the cellulosic fibrous product (a) a compound of the formula



wherein R is an organic hydrophobic hydrocarbon group, R' is selected from the group consisting of hydrogen, methyl, and chloromethyl, and n is an integer of from 0 to 2, and (b) a polyalkyleneimine having from 2 to 3 carbon atoms in each alkylene group, the combined amounts of (a) and (b) being about 0.01% to about 5% of the weight of the dry cellulose fibers, and the weight proportions of (a) to (b) being from about 1:10 to about 10:1, and drying the thus treated cellulose fibrous product.

7. A method as described in claim 6 wherein an aqueous cellulosic pulp dispersion is treated with an emulsion of compound (a) in which R is an alkyl group having at least 10 carbon atoms, R' is hydrogen, and n is 2, and (b) an aqueous dispersion of polyethyleneimine.

8. A method as described in claim 6 wherein an aqueous cellulosic pulp dispersion is treated with an emulsion

of compound (a) in which R is an alkyl group having at least 10 carbon atoms, R' is chloromethyl, and n is 2, and an aqueous dispersion of polyethyleneimine.

3,310,460 3/1967 Goldstein et al. ----- 162—164  
3,345,251 10/1967 Gaertner ----- 162—158

S. LEON BASHORE, Primary Examiner

5 F. FREI, Assistant Examiner

U.S. CL. X.R.

References Cited  
UNITED STATES PATENTS  
2,961,367 11/1960 Weisgerber ----- 162—168X  
3,016,325 1/1962 Pattilloch ----- 162—168X

8—116; 117—155; 162—182